

Patented May 5, 1925.

1,536,151

# UNITED STATES PATENT OFFICE.

MARIA SCHOLZ, OF LEICHLINGEN, GERMANY.

## PROCESS FOR DYEING TEXTILE FABRIC, PAPER, AND LIKE MATERIALS.

No Drawing.

Application filed June 25, 1923. Serial No. 647,759.

*To all whom it may concern:*

Be it known that I, MARIA SCHOLZ, a citizen of Germany, residing at Leichlingen, Rhenish Prussia, Germany, have invented 5 certain new and useful Improvements in Processes for Dyeing Textile Fabric, Paper, and like Materials, for which I have filed an application for Letters Patent in Germany, August 12, 1922, and of which the following is a specification.

In the art of dyeing textile fabrics, paper, and like materials, the dye stuff is generally fixed by treating the dyed material within a steam chamber or by the well known Mather-Platt process. These procedures take time and are expensive, as complicated and bulky apparatus and a relatively large amount of steam is required; furthermore, a uniform fixation throughout 20 the material cannot be depended upon, and goods of inferior quality are often the result.

The object of the present invention is to turn out a high grade of dyed goods at a great reduction in time and costs by a new process of fixing the substantive, basic, acid or other dyestuffs previously applied to the fabric in any suitable manner.

My invention broadly consists in suitably dyeing the fabric, and in then fixing the color by means of an oleaginous agent at effective temperatures, which in the present instance means temperatures around 80 to 100 degrees Celsius, and in then finally removing the fixing medium again from the fabric and after-treating the latter in any required manner.

I have found that vegetable oils, such as for instance olive oil, can well be used for this purpose, but also the less expensive mineral oils of various grades of volatility are eminently suitable. In choosing the oleaginous substance best suited in each particular case, among other factors, the porosity of the material to be treated, the lighter or darker color shades obtaining, and the chemical nature of the dyestuffs and other agents entering into the several steps, must be carefully considered.

Good results have been obtained with paraffin oil, refined petroleum oils, and other mineral oils of a boiling point between 160 to 220° C. and by employing the oil bath at temperatures ranging from 80 to 100° C.

After the cloth or other porous material has been suitably dyed by imprinting,

spraying, stenciling, or in any other suitable manner with an aqueous solution of the dyestuff, the fabric is, preferably without delay, passed through a bath of the oleaginous agent heated to about 80 to 100° C. when the fixing of the color or colors will be properly effected within a relatively very short time, one minute being sufficient in most cases. The fixing agent is then removed again from the fabric by squeezing, drying and evaporating, and it may be readily recovered for further use in well known manner. The fixed goods are then washed and, if required, after-treated in suitable manner well known in the art.

In the case of cloth printing the padding machine may be used for applying the dyeing medium, whereupon the dyed stuff is best at once, in a more or less wet state, passed through the hot fixing bath, which latter should be kept at a temperature of around 90° C.

If the stated steps are followed, the dye will properly be fixed without precipitation of sediment in the fixing bath.

The advantages obtained by the described process will be readily understood from a comparison with the prior dyeing and fixing art. When using basic dyeing agents the prior steps for making the goods color-fast to washing consisted in first treating them with acid mordants, such as tannin or tannic acid, then dyeing and steaming them, and finally treating them with tartar emetic. In this treatment tannin lake is formed which fixes the basic dyes and thus makes them water-fast. I now have found that the same results can be obtained at greatly reduced costs and without entailing time-consuming preliminary and after-treatments, by subjecting the goods to the above described action of a hot oil bath.

I have further found that in the case of discharge-printing where first the dye and next the discharge is applied, the goods thus prepared can be fixed and the discharge be made effective in a single operation in the same oleaginous substance, the fixing and discharging period taking not over one minute, whereas in the prior art the fixing of the dye and the discharging had to be done by separate successive treatments.

Stuffs dyed according to my new method are not only fast to rubbing and fast to washing in the ordinary sense of this latter term, but they are also fast to drops fall-

ing on them, and, furthermore, the discharges produce perfect white patterns.

My new process can advantageously be used also for improving goods previously dyed by other processes, by rendering them still more water-fast, drop-fast, and unaffected by rubbing. This, in itself, is of great moment since it is now possible to use dyestuffs of inferior and cheaper quality 10 with equally good results in the finished product.

My new process can also be used with particular good results in the case of heavy fabrics, such as plush, felt, velvet and the 15 like, which heretofore required a relatively very extended dyeing treatment for obtaining permanent colors.

By reason of the speedy and thorough fixing effect of my hot oil bath the complete 20 dyeing operation is considerably curtailed and is performed at lower temperatures than heretofore, all of which makes for a substantial saving in time, labor, and fuel.

When using the term "dyeing" in the 25 foregoing specification and in the appended claims, I want it to be distinctly understood that this term is to include broadly any steps known to those skilled in the dyeing and printing art for applying to the material coloring, mordanting, thickening and other matter, whether this is to be done in or several operations, the particular feature claimed by me residing substantially in the 30 step of passing a material, dyedly pretreated in any suitable manner, through a hot oil bath within which the colors are effectively fixed in a relatively very short time.

What I claim is:—

1. The described step in the art of dyeing 40 textile and other porous material, which consists in steeping the dyed material in a quick-acting hot fixing liquor.
2. The described step in the art of dyeing 45 textile and other porous material, which consists in passing the dyed material through a quick-acting hot oil bath.

3. The described process of dyeing textile and other porous material, which comprises dyeing the material and then treating it in a hot bath of oleaginous character. 50

4. The described process of dyeing textile and other porous material, which comprises causing an aqueous solution of the dyestuff to act on the material and then passing the still moist material into a hot oil 55 bath.

5. The described process of dyeing textile and other porous material, which comprises dyeing the material and then treating it in an oleaginous substance heated to effective 60 fixing temperatures, and in subsequently removing again said oleaginous substance from the material.

6. The described process of dyeing textile and other porous material, which comprises 65 dyeing the material and then passing it through a bath of hot mineral oil.

7. The described process of dyeing textile and other porous material, which comprises dyeing the material and then passing 70 it through a bath of mineral oil heated to a temperature within the limits of 80 to 100° C.

8. The described process of dyeing textile and other porous material, which comprises 75 dyeing the material and then passing it through a bath of refined mineral oil having a boiling point range of between 160 to 220° C. and heated to a temperature substantially lower than the lowest degree of 80 said boiling point range.

9. The described process of dyeing textile and other porous material, which comprises dyeing the material, passing it through a 85 bath of mineral oil having a boiling point range of between 160 to 220° C. and heated to a temperature of between 80 to 100° C., and subsequently removing the said oil from the material.

In testimony whereof I affix my signature.

MARIA SCHOLZ.